

1

2,774,232

## METHOD OF MANUFACTURING SILK STOCKINGS

Hisashi Kakizaki, Suwa, Nagano Prefecture, Japan

No Drawing. Application March 5, 1951,  
Serial No. 214,017

Claims priority, application Japan June 9, 1950

4 Claims. (Cl. 66—178)

This invention relates to method of manufacturing of 15 stockings, in particular knitted silk stockings.

The reason why silk stockings are weaker than nylon stockings results from the fact that in the course of refining silk the latter remains in the state of fibers. The bundle of these fibers expands during the treatment to the extent that its apparent diameter becomes larger than actually desired. In other words, ladies who desire to wear thinner stockings nowadays, cannot resort to silk stockings made from very thin fibers due to the particular structure of the raw silk. As the raw silk is generally made up from several cocoon threads embracing one another, the outer appearance thereof seems to be comparatively fine.

However, if such raw silk is refined, sericin is removed and its increased diameter not only becomes from 1.3 to 1.5 times the diameter of raw silk but also the cocoon threads composed of two fibroin fibers closely adhered by sericin separate from each other upon removal of sericin, and therefore raw silk will generally be composed of very fine fibroin fibers only. Particularly in case of thin silk stockings contraction of the fibers often occurs which causes easy breakage of and damage to silk stockings. This is one of the reasons why a "run" occurs more easily with silk stockings than with nylon stockings.

The following table shows the comparison of the actual diameter with the increased diameter of a bundle of raw fibers used in silk stockings and nylon stockings, which will give an idea why silk stockings hitherto manufactured are relatively weak.

Table I

| Marks | Kind of Materials | Actual diameter of a bundle of raw fibers, D in microns | Increased diameter of a bundle of raw fibers, D <sub>1</sub> in microns | D <sub>1</sub> /D | Deniers of raw fibers | No. of twist per meter                   |
|-------|-------------------|---------------------------------------------------------|-------------------------------------------------------------------------|-------------------|-----------------------|------------------------------------------|
| F-7   | Silk              | 83.5                                                    | 128.0                                                                   | 1.525             | 42                    | 600, clockwise.                          |
| N-12  | Nylon             | 91.4                                                    | 127.0                                                                   | 1.390             | 51                    | 380, counterclockwise.                   |
| H-4   | Silk              | 100.0                                                   | 150.0                                                                   | 1.500             | 56                    | 1,300 clockwise, 1,500 counterclockwise. |
| N-2   | Nylon             | 112.0                                                   | 150.0                                                                   | 1.340             | 63                    | 360, counterclockwise.                   |

NOTE.—In the above items "a bundle of raw fibers" means raw fibers used for the leg part of stockings.

In Table I, F-7 and N-12 or H-4 and N-2 designate respectively stockings having approximately the same appearance of thinness. Comparing two pairs of stockings of each kind, it will be seen that the deniers of nylon are 51 in N-12 or 63 in N-2 whereas the deniers of silk are 42 in F-7 or 56 in H-4, that is, the actual diameter of a bundle of fibers of nylon stockings is always larger than that of silk stockings. This is one of the reasons why nylon stockings are stronger than silk stockings. For the purpose of comparison, the silk fiber has a heavy twist of 600 per meter in F-7 and 1,500

2

turns per meter in H-4 whereas the nylon fiber has a light twist of 380 per meter in N-12 and 360 per meter in N-2 so that the raw silk fiber ought to appear considerably fine as compared with nylon fibers. Contrary to this expectation, the silk fiber has, however, a relatively very thick appearance in comparison with the nylon fiber. This is a great disadvantage of the silk fiber.

In case when contraction in thin stockings of either silk or nylon is caused, it is difficult to arrive again at the original thread or fiber structure due to the twist imparted thereto. Therefore, it is advisable to prefer fibers with a light twist, but up to now, the method of manufacturing silk stockings required a heavy twist to the fiber because the increased diameter of a bundle of raw fibers does not become fine without giving a heavy twist to such fibers.

When all-silk stockings are refined, the rate of refining of the leg part with coarse mesh of fine raw silk is greater than that of the welt, heel, sole and toe parts with fine mesh of thick raw silk. Thus, the leg part is too refined and the bundle of fibers heavily expands to cause the easy generation of contraction.

If the part of coarse mesh can be refined as well as the part of fine mesh at the same rate, the leg part will not be too refined. Consequently, the object of the invention is to obtain the rate of refining by means of heretofore known treatment of raw fibers for the leg part with formalin or other chemicals to lower the solubility of sericin. Further, it is contemplated according to the invention to more effectively produce silk stockings having equal durability to nylon stockings whereby the diameter of a bundle of fibers in silk stockings remains constant as to the magnitude of raw silk fibers.

If the process according to the invention is carried out along the above outline, that is to say, if silk stockings are refined after knitting operation by the use of raw silk for entire parts of welt, heel, sole and toe, and raw silk previously treated to fix sericin for the leg part, the result is obtained that the leg part remains in the same state of raw silk whereas the welt, heel, sole and toe parts become elastic and flexible due to the removal of sericin by a degumming operation.

Therefore, the raw silk fiber assumes substantially mass quality equal to that of the nylon fiber. Thus silk stockings as thin as possible may now be produced.

In short, this invention relates to a method of manufacturing silk stockings which is characterized by knitting them from raw silk which is previously treated to fix sericin for the leg part and to soften the fibers employed for the welt, heel, sole and toe parts. Several ways suitable for carrying out the process described above are given in the following examples.

For shortness' sake hereafter the welt, heel, sole and toe parts are described as A and the leg part as B.

Example 1.—Ordinary raw silk is used for A and raw

silk previously treated to fix sericin for B. After knitting only sericin of A is removed.

*Example 2.*—Raw silk previously refined about seventy percent is used for A and ordinary raw silk for B. After knitting raw silk for A is slightly softened.

*Example 3.*—Raw silk of fibroin fibers only by previously refining is used for A and silk which is suitably twisted and previously treated to fix sericin for B. After knitting raw silk fibers are finished before or after dyeing without special refining.

*Example 4.*—Nylon, "Vinyon" (of the formula



cotton, artificial silk, staple fiber or other soft fibers as well as silk which is suitably twisted and previously treated to fix sericin, are used for A, and soft raw silk fibers having the same diameter of a bundle of fibers as that of raw silk and the small increased diameter by means of refining raw silk previously in such a degree that defects do not appear, i. e., 50% refining to remove about 10% of sericin and afterward treatment to fix sericin, or silk which is suitably twisted and previously treated to fix sericin, are used for B, and then stockings are knitted.

*Example 5.*—By combining raw silk fibers for B described in Example 4 with each of raw fibers for A described in Examples 1 to 4, silk stockings are knitted from these fibers.

The result of experiment on the stockings produced by the process described in Example 1 is shown in the following table:

Table II

| Marks | Kind of fibers | No. of filaments | Actual diameter of a bundle of fibers, D in microns | Increased diameter of a bundle of fibers, D <sub>1</sub> in microns | D <sub>1</sub> /D | Deniers of raw fibers | No. of Twist per meter                      |
|-------|----------------|------------------|-----------------------------------------------------|---------------------------------------------------------------------|-------------------|-----------------------|---------------------------------------------|
| N-4   | Nylon          | 10               | 77.5                                                | 87.5                                                                | 1.130             | 43.4                  | 1,400                                       |
| K-6   | Silk           | 16               | 80.4                                                | 88.7                                                                | 1.102             | 45.0                  | Without twist.                              |
| F-16  | Silk           | 30               | 75.0                                                | 114.0                                                               | 1.520             | 42.0                  | 1,300 counterclockwise.<br>1,600 clockwise. |

NOTE:

1. F-16 is ordinary silk stockings and K-6 silk stockings produced by the process of this invention.  
2. No. of filaments per meter of K-6, i. e. 16, means No. of cocoon threads, because two fibers are adhered to one piece of sericin.

As shown in Table II, deniers of raw fibers of both N-4 and F-16 are about 43 and their actual diameters of a bundle of fibers are approximately the same. However, the actual diameter of a bundle of silk fibers is 114.0 microns whereas that of nylon fibers is 87.5 microns. Therefore, the ratio of D<sub>1</sub> to D of F-16 is 1.520 and of N-4 1.130 respectively, and both have the same heavy twist. Comparing K-6 produced by this process with N-4, it will be seen that both have approximately the same apparent diameter of a bundle of fibers, their thicknesses are relatively thin of the same grade, and deniers of K-6 are 42, whereas those of N-4 are 43.4, so that the raw fiber of K-6 has the larger substantial mass than that of N-4. It follows that if the raw fiber of K-6 is given a suitable twist, it will provide for a larger substantial mass than that of nylon which is given

a heavy twist of 1,400 per meter. It is known that contraction occurs in silk stockings rather than in nylon stockings whereby in silk stockings contraction causes always a "run." However, there seldom occurs contraction in the stockings manufactured according to the method of this invention, because the bundle of fibers remain in the same state of raw silk even if refined and when washed after knitting in view of the treatment to fix sericin. Therefore, so called "run-proof" silk stockings can be obtained according to the invention.

Having thus described the invention, what is claimed as new and desired to be secured by Letters Patent, is:

1. The method of manufacturing hose substantially from raw silk fibers, comprising the steps of knitting raw silk fibers previously treated to fix sericin therein to thereby obtain a major part of said hose, and then knitting previously degummed raw silk fibers to attain the remainder of said hose, whereby said remainder of said hose presents elasticity and flexibility relatively higher than said major part of said hose.
2. The method of manufacturing hose substantially from raw silk fibers, comprising the steps of knitting raw silk fibers previously treated to fix sericin therein to thereby obtain the leg part of said hose, then knitting raw silk fibers to attain the remainder of said hose, and finally removing sericin from said latter raw silk fibers by degumming operation, whereby said remainder of said hose presents elasticity and flexibility relatively higher than said leg part of said hose.
3. The method of manufacturing a knitwear product, comprising the steps of knitting raw silk fibers, previously treated to fix sericin therein to thereby obtain a

major part of said product, and then knitting the remainder of said product from a previously refined fiber, whereby the remainder of said product presents elasticity and flexibility relatively higher than said major part of said product.

4. The method of manufacturing hose, comprising the steps of knitting raw silk fibers, previously treated to fix sericin therein into the leg part of said hose, and then knitting the remainder of said hose from a soft, previously refined fiber of silky texture.

References Cited in the file of this patent

UNITED STATES PATENTS

- 2,029,972 Wallerstein et al. Feb. 4, 1936  
2,040,736 Goodman May 12, 1936  
2,503,444 Lawson et al. Apr. 11, 1950